

# UNITED STATES PATENT OFFICE.

ROBERT M. KEENEY AND LOUIS F. VOGT, OF WASHINGTON, PENNSYLVANIA,  
ASSIGNORS TO STANDARD CHEMICAL COMPANY, OF PITTSBURGH, PENNSYLVANIA.

## NICKEL-URANIUM ALLOY.

1,240,055.

Specification of Letters Patent. Patented Sept. 11, 1917.

No Drawing.

Application filed December 24, 1915. Serial No. 68,543.

To all whom it may concern:

Be it known that we, ROBERT M. KEENEY and LOUIS F. VOGT, citizens of the United States, and residents of Washington, in the county of Washington and State of Pennsylvania, have invented certain new and useful Improvements in Nickel-Uranium Alloys; and we do hereby declare the following to be a full, clear, and exact description 10 of the invention, such as will enable others skilled in the art to which it appertains to make and use the same.

This invention relates to an improvement in alloys,—the object of the invention being 15 to produce a nickel-uranium alloy in which a relatively large proportion of uranium may be effectually alloyed with the nickel.

With this and other objects in view, the invention consists in a combination of alloyed metals as hereinafter set forth and pointed out in the claims.

The materials which we employ in the manufacture of nickel-uranium are uranium, preferably in the form of uranium oxide, 25 fluorspar as a slag-forming material; a carbonaceous reducing agent, preferably petroleum coke containing at least seventy per cent. fixed carbon, and nickel in a finely divided condition. All of these materials 30 should be as free as possible from impurities, especially silica or silicon.

We mix the finely divided nickel with uranium oxide or sodium uranate. For example, in a 30 per cent. uranium product, we 35 prefer to use the proportions approximately of 1 lb. of nickel to six-tenths of a pound of uranium oxide ( $U_3O_8$ ). At the same time we mix in carbonaceous material (petroleum coke for example) containing at least 70 per 40 cent. of fixed carbon. To this mixture of nickel, uranium oxide, and carbon, we add fluorspar in the proportions, approximately, of eight-tenths of a pound of fluorspar to one pound of nickel. The mixture thus 45 formed is charged into an electric furnace at a rate dependent upon the size of the furnace and the grade of alloy being made, but in no case should the mixture be charged so fast as to cool the furnace to any great degree. Regular intervals of charging is a 50 matter of considerable importance. In other words, a charge should be introduced into the furnace as soon as a previous charge

has been reduced and melted. In the operation of the furnace, a portion of the charge 55 will collect on the wall of the furnace and affords a protection to the lining,—the charge thus forming, in effect, a lining in the furnace.

The reactions involved are those of simple 60 carbon reduction, the reduced uranium alloying with the nickel to form a nickel-uranium alloy.

We have found that fluorspar is the best and probably only slag-forming material 65 which may be successfully used to obtain a reasonable proportion of uranium in the alloy, and it should be used in considerable quantity, and be of a high grade so as to avoid impurities which would be detrimental 70 to the alloy.

A typical charge for the production of nickel-uranium (the uranium oxide containing 68.8 uranium or 82 per cent.  $U_3O_8$ ; the coke 70 per cent. fixed carbon; the nickel 75 (low in impurities) may be substantially as follows:—

|                       |     |      |
|-----------------------|-----|------|
| Finely divided nickel | 10  | lbs. |
| Uranium oxide         | 7.5 | lbs. |
| Coke                  | 6   | lbs. |
| Fluorspar             | 8   | lbs. |

Of the uranium put into this charge, at least 75 per cent. will be contained in the finished alloy. One hundred pounds of the 85 said charge will produce approximately forty pounds of nickel uranium, and by remelting the residue approximately 85 per cent. of the uranium would be alloyed with the nickel and about 45 pounds of nickel- 90 uranium obtained.

The nickel-uranium made from the typical charge above stated will contain ingredients approximately in the following proportions

|    |      |           |
|----|------|-----------|
| U  | 29.2 | per cent. |
| C  | 5.12 | per cent. |
| Si | 2.68 | per cent. |
| Ni | 63.  | per cent. |

Having fully described our invention what we claim as new and desire to secure by Letters-Patent, is:—

1. A nickel-uranium alloy containing more than twenty-five per cent. uranium.
2. A nickel-uranium alloy containing be-

tween twenty-five and thirty per cent, uranium and more than sixty per cent. nickel.

3. An alloy consisting substantially of nickel and uranium, the uranium content being approximately one-half as much as the nickel.

In testimony whereof, we have signed this

specification in the presence of two subscribing witnesses.

**ROBERT M. KEENEY.**  
**LOUIS F. VOGT.**

Witnesses:

**R. E. LAURENCE,**  
**A. D. RILEY.**